

Nov. 2, 1937.

G. LUTZ

2,097,630

PLATING OF CADMIUM

Filed Oct. 17, 1935



INVENTOR.

GEORGE LUTZ.

BY

Albert B. Briggs.

ATTORNEY.

## UNITED STATES PATENT OFFICE

2,097,630

## PLATING OF CADMIUM

George Lutz, Rocky River, Ohio, assignor, by  
mesne assignments, to E. I. du Pont de Nemours & Company, Wilmington, Del., a corporation of Delaware

Application October 17, 1935, Serial No. 45,426

17 Claims. (Cl. 204—1)

This invention relates to the electrodeposition of cadmium from cyanide-cadmium baths, and is particularly directed to cyanide-cadmium plating compositions, plating baths, and plating processes which employ, as an addition agent, a reduced amketaldoresin whereby a bright, smooth, uniform cadmium deposit is obtained.

It has heretofore been proposed to modify the character of cadmium deposits by the use of organic addition agents such as sulfite cellulose waste, dextrin, starch, alkylated naphthalene sulfonic acids, wool, caffeine, shellac casein, licorice, glucose, alkali reaction products of heterocyclic aldehydes, furfural, gum arabic, and gelatine.

It has been necessary to employ an addition agent and/or a brightener with cyanide-cadmium plating baths, because, without such modifying agents, cadmium deposits of exceedingly poor character and appearance are obtained. The properties of electrodeposited cadmium are largely determined by the addition agent and/or brightener used, and the desirability of a cadmium plate is, to a great extent, dependent upon the efficacy of the modifying agents employed.

The properties of a cadmium plate are partly dependent, in commercial practice, upon certain characteristics of the plating bath employed, and these characteristics can be modified, to some extent, by suitable organic addition agents and/or brighteners. Under strictly controlled conditions, one can deposit a fairly satisfactory cadmium plate on a flat cathode with a bath which, in ordinary commercial practice, would be unsatisfactory. Under the usual conditions of commercial operation, particularly when recessed articles or articles of irregular shape are to be plated, a bath must have a fairly wide bright current density range and good throwing power if even moderately satisfactory results are to be obtained. The throwing power and the extent of the bright range have been somewhat improved by the use of the addition agents heretofore known.

While the addition agents hitherto employed have effected a considerable improvement in processes for the electrodeposition of cadmium, the results obtained have not been all that could be desired.

I have found that the reduction products of certain derivatives of ketaldones are exceedingly effective addition agents for cyanide-cadmium plating. By the use of these novel addition agents, it is possible to electrodeposit cadmium from cyanide-cadmium baths as a bright, smooth, lustrous, ductile, adherent deposit. Baths containing these novel addition agents are characterized by good throwing power and by a wide bright current density range.

In the accompanying drawing there are shown

the relationships existing between various derivatives which constitute the addition agents of my invention, and there are also shown, diagrammatically, the methods of preparation of the various derivatives.

Represented by a circle in the upper left-hand corner of the drawing are the starting materials from which my addition agents are derived. The starting materials are designated "ketaldones" but, as will be explained below, certain ketaldones are particularly suitable for my purpose.

My preferred starting materials are, generally speaking, aliphatic and carbocyclic ketaldones, that is aldehydes and ketones, but, as will become apparent hereinafter, the best results are obtained by the use of certain aliphatic and carbocyclic aldehydes and ketones.

The term "ketaldonyl" has been applied to designate the  $C=O$  group as it appears in aldehydes and ketones in contradistinction to the  $C=O$  group as it appears in acids. Of course, the carbonyl group as it appears in acids,



25

is very different in its properties from the carbonyl group as it appears in aldehydes and ketones, and the expression "ketaldonyl group" is employed to distinguish the aldehydic and the ketonic carbonyl group from the acidic carbonyl group. The expression "ketaldonyl group" as used herein designates a carbonyl group in which a third carbon valence is joined to carbon and in which the remaining valence is satisfied by carbon or by hydrogen. Or, in chemical symbols, the "ketaldonyl group" as used herein is of the type



40

wherein R is a hydrocarbon radical and where R' is hydrogen, in the case of an aldehyde, or R' is a hydrocarbon radical, in the case of a ketone. It will also be understood that the ketones and aldehydes themselves are referred to herein as ketaldones in accordance with this terminology.

The starting materials which I employ are, broadly, ketaldones. While I may use aldoses, ketoses, heterocyclic aldehydes and ketones or any other such ketaldones, I prefer to use aliphatic and carbocyclic ketaldones which do not contain a carboxyl group, which do not contain sulfur, and which do not contain nitrogen. The starting materials, moreover, should contain no more than two hydroxyl groups and preferably should contain at least two carbon atoms. More specifically, I prefer to employ

50

55

60

ketaldones which contain only carbon, hydrogen, and oxygen, which contain at least two carbon atoms, and in which the hydrogen-oxygen ratio is greater than that of water.

5 As is illustrated in the drawing, the starting materials, the ketaldones, are reacted with ammonia or an amine, in alkaline solution, to produce an amo-reaction product. It will be observed that "amo" is used to designate both ammonia and an amine. As will be noted hereinafter, the amo-reaction products of the ketaldones are very similar in their physical and chemical characteristics. They all contain nitrogen, and all are, apparently, complex mixtures. I have, 10 accordingly, designated these reaction products "amketaldoresins". The nature of the products and the nature of the reaction will be discussed in more detail hereinafter.

The amketaldoresins are subsequently modified 20 by hydrogenation to yield nitrogen-containing derivatives which are effective as addition agents. These derivatives, while more effective, are very similar to the amketaldoresins, ordinarily differing slightly as to color and solubility.

25 A preferred group of ketaldones, the aldacet, are illustrated in the upper right-hand corner of the drawing. More will be said hereinafter regarding the members of the illustrated aldacet equilibrium. As is shown in the drawing, the aldacet, like the ketaldones generally, are reacted with ammonia, or cyanide to produce an amketaldoresin. The particular amketaldoresin produced from the aldacet are designated herein, the "amaldacets."

30 35 According to my invention, the amaldacets are hydrogenated, as were the amketaldoresins generally, to produce nitrogen-containing derivatives.

The ketaldones which I employ as starting materials are reacted in weak alkaline solution with an amo to produce an amo-reaction product from which addition agents of my invention may be prepared. As will be noted hereinafter, the use of cyanide is considered substantially equivalent 40 to reacting the ketaldones with amoes in alkaline solution.

45 The amketaldoresins are preferably derived from the aliphatic ketaldones termed the aldacet. The derivatives of the aldacet are typical of the amketaldoresins, and their preparation will be described below in some detail as illustrative of the amketaldoresins generally.

The aldacet comprise the aliphatic aldehydes: 50 acetaldehyde, aldol, crotonaldehyde, and paraldol. In dilute alkaline solution the aldacet appear to exist in equilibrium, any one of the aldacet leading to the production of all at a rate of conversion apparently depending upon the specific aldacet first present. The aldacet equilibrium is illustrated in the upper, right corner of the drawing.

55 Referring to the aldacet equilibrium in more detail, it is noted that acetaldehyde in dilute alkaline solution is quickly converted to aldol thus:



65 The aldol may lose one molecule of water and become crotonaldehyde, thus:



The aldol may condense to form paraldol, thus:



The  $n$  in Equation 3 is a whole number, probably 2.

5 In order to visualize the relationships existing between the aldacet, reference should be had to the accompanying drawing wherein these relationships are diagrammatically illustrated. It is to be understood that the relationships are shown with reference to the compounds in dilute alkaline 10 solutions or in alkali metal cyanide solutions.

15 In the drawing, acetaldehyde is illustrated as converting to aldol. The aldol may go to paraldol or to crotonaldehyde. The aldol might also go back to acetaldehyde, but only to a small extent. The paraldol may go back to aldol, or it may lose 20 water and go to crotonaldehyde, though this latter conversion probably takes place to a very small degree. The crotonaldehyde may form from acetaldehyde, aldol, or paraldol, and, by gaining water, may revert to any of them, though it is likely that it would move largely by way of aldol.

25 As is seen in the drawing, then, we may consider the aldacet as being in equilibrium. This equilibrium will, according to my belief, be substantially the same regardless of which of the four substances are initially added to the cyanide solution, though, as will hereinafter be noted, the aldacet are not entirely equivalent, and it is possible that some of the aldacet in dilute alkaline solution form this aldacet equilibrium rather slowly or move more rapidly in certain directions than in others.

30 While I have mentioned only acetaldehyde, aldol, crotonaldehyde, and paraldol as members 35 of this sub-genus, I may use any condensation product of acetaldehyde in dilute alkali solution. Another aldacet is paraldehyde. Ordinarily paraldehyde is considered as forming only in acid 40 solution, but I have reason to believe that at least some paraldehyde forms in the discussed aldacet equilibrium. Paraldehyde is apparently very slow to convert to other aldacet and probably because of this fact is none too satisfactory as a starting material.

45 Aldol, acetaldehyde, crotonaldehyde, and paraldol are the only commercially available aldacet at the present time. For practical reasons, therefore, I prefer to use as a starting material an aldehyde selected from the group consisting of 50 acetaldehyde, aldol, crotonaldehyde, and paraldol.

55 It is to be noted that the aldacet are those aliphatic ketaldones, such as acetaldehyde, aldol, crotonaldehyde, and paraldol, which exist in some sort of equilibrium when one of the said ketaldones is put into alkaline or alkali metal cyanide solution. Generally, then, one might say that the aldacet are aliphatic aldehydes from the group consisting of acetaldehyde and its condensation or equilibrium products in alkaline and 60 alkali metal cyanide solutions.

65 As a definition for the purposes of this application, then, the aldacet are reversible equilibrium-condensation products of acetaldehyde in alkaline solution and particularly in alkaline solutions such as those of the following Examples I and X.

70 As will be noted in detail hereinafter, the aldacet are not entirely equivalent for my purposes but are substantially so. Crotonaldehyde, for example, seems to lead to slightly lower yields. This may be attributable to the fact that crotonaldehyde is but slowly converted to the necessary form, or to some other now unknown cause.

75 As is above indicated, there is considerable uncertainty as to the extent and nature of the

conversion of some aldacones to others. All of the evidence now available to me substantiates the putative theory above advanced as to the nature of the aldacon equilibrium, but it will be understood that direct experimental evidence is obtainable only with great difficulty. In most instances the aldacon equilibrium exists for only a short time, some further action quickly taking place to form resins. That the aldacones are in some kind of equilibrium is relatively certain, but the proportions of individual aldacones and the rates of conversion have, to date, defied exact determination.

It is clearly to be understood that the above description of the relations between the initial materials is for purposes of illustration and that I do not intend to be limited in any way thereby, because the chemistry of these compounds is intricate and obscure, and because my results are obtained entirely apart from theoretical considerations. It is also to be understood that while I refer to aldol, acetaldehyde, crotonaldehyde, and paraldol as resulting from the condensation of acetaldehyde in alkaline solutions, I do not wish to be limited thereby, as I may use aldol, acetaldehyde, crotonaldehyde, and paraldol which have been made in any manner.

Turning now to a consideration of the amketaldoresins produced from the aldacones, it is first noted that the specific amketaldoresins produced by the reaction of the aldacones with amines or cyanide in alkaline solutions are termed "amaldacets." The amaldacets are almost indistinguishable from one another in physical and chemical properties though, as will be noted herein-after, they differ slightly from one another as to their efficiency as addition agents for cyanide-cadmium plating.

It is to be noted that the term "reaction" is used to express whatever occurs when the ketaldones, or specifically the aldacones, are treated in alkaline solution with cyanide or with an amine. The term "reaction" is used to distinguish from "condensation" as used above with reference to the aldacon equilibrium tho, in fact, the reaction probably includes both polymerizations and condensations.

The amaldacets as well as the amketaldoresins contain nitrogen as determined by the Kjeldahl method. In the amaldacets the nitrogen is present in about the ratio of one nitrogen atom to each two molecules of aldol (four of acetaldehyde, one of paraldol, etc.). I have been unable to determine how the nitrogen is located in the amaldacet molecules, and insufficient evidence is available to warrant any assumptions.

That the amaldacets are not simple compounds, but are complex mixtures, is evidenced by the fact that portions are water-soluble, other portions are chloroform-soluble, etc. It seems probable that the amaldacets are the result of many intricate polymerizations, condensations, and reactions. There may be some condensation products which are not combined with nitrogen, but the fact that a molecular proportion, or an excess, of an amine or of an alkali metal cyanide, to aldehyde give the best results, leads to the belief that the amount of such uncombined products is relatively small.

The reaction which leads to the amaldacets takes place, I believe, between ammonia, an amine, or possibly  $CN^-$  and one or more of the amaldacets. This reaction is illustrated in the drawing by dashed lines. The aldacon, or aldacones, which react with the nitrogen compound may go first to some other and unknown form

and then react. I conceive of the reaction as withdrawing one, or more, of the aldacones from the equilibrium with the result that the remaining aldacones move towards the removed materials to restore the equilibrium, and are so all 5 finally utilized.

I have reason to believe that two or more of the materials in equilibrium react with cyanide to produce the final product, or else the one which reacts with the cyanide moves through a number 10 of different paths to produce a number of final products. This is evidenced by the fact that the reaction product is a mixture of separable materials. More is said of this separability hereinafter.

To illustrate the production of the amaldacets 15 by the reaction of aldacones with ammonia or amines, the following specific examples are given:

#### Example I

Equimolecular proportions of crotonaldehyde 20 and monoethanolamine were reacted, starting the reaction at room temperatures. The temperature of the mixture was held at about forty to fifty degrees centigrade until no further reaction 25 was apparent. The reaction mixture was a red-dish-brown, viscous liquid, readily soluble in cyanide-cadmium plating baths.

#### Example II

A similar amaldacet was produced by reacting 30 equimolecular proportions of aldol and monoethanolamine. A product exceedingly similar to the one of Example I was produced.

#### Example III

One-half mole of monoethanolamine and one mole of aldol were reacted at temperatures between 30 and 40° C. The product was not as soluble as the product of Example II and, when reduced, it was not as satisfactory an addition 40 agent for use in cyanide-cadmium plating.

#### Example IV

Equimolecular proportions of aldol and diethanolamine were reacted at room temperatures. 45 A product very similar to those of the above examples was produced, the product of this example, however, being slightly less soluble than the product of Examples I and II.

#### Example V

Equimolecular proportions of aldol and triethanolamine were reacted at room temperatures. The reaction product of this example was somewhat less soluble than the products of Examples 55 I and II.

#### Example VI

Aldol was treated with ammonia gas by bubbling 60 the gas through the aldol until no further reaction was noted. The reaction product, when reduced, was rather difficultly soluble, and was only a moderately efficient addition agent for cyanide-cadmium plating baths.

#### Example VII

Equimolecular proportions of crotonaldehyde and ammonium hydroxide were reacted. The reaction product was very similar to that of the preceding example. After several days, the 70 amaldacet of this example solidified, becoming much less soluble.

#### Example VIII

Crotonaldehyde and ammonia gas were reacted 75

at about twenty-five degrees centigrade. The product was very similar to that of the preceding example. After a few days the product of this example solidified to a brittle, red resin.

5

*Example IX*

Acetaldehyde was treated with an excess of gaseous ammonia. An amaldacet similar to that of the preceding example was obtained.

19 While I have shown the reaction of the aldacet with ammonia, ammonium hydroxide, and with certain amines in the above examples, it will be understood that other amines may be used. I may, for instance, prepare the amaldacets by treating 15 the aldacet with amines such as the glucamines, for instance, glucamine and methyl glucamine, or aliphatic amines, for instance, methyl ethylamine, methylamine, and ethylamine.

20 While the amaldacets may be prepared by conducting the reactions of the above examples at rather widely varied temperatures, I prefer that the reaction be performed at temperatures between about thirty and fifty degrees centigrade. If much lower temperatures be maintained, the 25 reaction products will tend to contain insoluble or relatively inactive constituents. Similarly, the reaction temperatures should not be permitted to rise too high, because, when the reaction proceeds at high temperatures, the reaction product may contain insoluble constituents and 30 may have none too great an efficiency as an addition agent.

35 It is generally preferred to employ an equimolecular proportion, or an excess, of amine to aldehyde. As will be noted by comparing Examples II and III, less satisfactory amaldacets are produced when less than an equivalent amount of amine is used.

40 Instead of preparing the amaldacets by the direct reaction of ammonia or amines with the aldacet, they may be prepared by reacting the aldacet with alkali cyanides.

45 When the aldacet are treated with liquid hydrocyanic acid, some slight reaction apparently occurs, but the product has but little, if any, activity as an addition agent in cyanide-cadmium plating baths, and hydrogenation according to my invention effects little improvement. From this fact it appears that when the aldacet are 50 reacted with alkali metal cyanides, no great portion of the reaction product contains the CN-group.

55 The cyanides are known to hydrolyze to produce ammonia and formates according to the following illustrative reaction:



It seems possible, accordingly, that the cyanide is hydrolyzed, and that the aldacet react with the 60 ammonia which is formed. This hypothesis is supported by the fact that the odor of ammonia is apparent throughout the reaction.

65 This hypothesis is further supported by the fact that the reaction products of the aldacet with amines and with cyanide are very similar.

While very similar, the reaction products of aldacet with alkali metal cyanides are somewhat more desirable than the reaction products of the aldacet with amines.

70 If, as I have assumed, the reaction with cyanide amounts to a reaction with ammonia by reason of the hydrolysis of the cyanide, it is surprising that such a difference in the amaldacets should exist. It seems possible, however, that the differences are attributable to the fact that in an alkali

metal cyanide solution the ammonia is somewhat less available. It is possible, of course, that some of the aldacet reacts with the cyanide directly or with some intermediate product of the hydrolysis. It seems probable, however, that the reaction occurs largely between the aldacet and the ammonia produced by hydrolysis of the alkaline cyanide solution.

5 75 The following specific examples illustrate the production of the amaldacets by the reaction of 10 aldacet with an alkali metal cyanide.

*Example X*

Five parts, by weight, of technical aldol were added to a solution containing three parts, by weight, of sodium cyanide in ten parts, by weight, of water. The reaction receptacle, to which the aldol was added, was provided with a water-cooling means, and convenient means were provided for heating the receptacle as required. By adding 20 the aldol slowly and employing the cooling means, the temperature of the reaction mixture was held between 45° to 50° C. This temperature was maintained for about two and one-half hours, cooling or heating the receptacle as required. As 25 the aldol was added, and for a time thereafter, the heat of the reaction necessitated a continuous cooling of the reaction mixture to hold the temperature within the desired limits. Later it became necessary to supply heat to the reaction 30 mixture to maintain the temperature. During the reaction a small amount of ammonia was liberated, as was evidenced by the characteristic odor.

The amaldacet-containing reaction mixture obtained may immediately be reduced to form one product of my invention. It is a thick, mobile liquid, dark red in color.

In order to purify and concentrate this reaction product, the solution, after being allowed to cool, was made neutral to litmus with a dilute solution of sulfuric acid. The acid solution consisted of one part by volume of water to one part by volume of concentrated sulfuric acid. There was then added an excess of ten per cent over the volume of dilute acid required to neutralize the solution. Sodium sulfate was precipitated, and the excess acid used depressed its solubility. The temperature was not allowed to go above 50° C. during this neutralization treatment. Hydrocyanic acid gas was evolved during the treatment and means were provided for disposing of it.

The acid treated solution was allowed to stand for several hours and a dark red fraction rose to the top. This top layer was removed and 55 centrifuged.

The separated top layer, which may be reduced to form a preferred product of my invention, is a viscous liquid, dark red in color, and it has a specific gravity of about 1.20. At temperatures as low as -17° C. it remains liquid, but at the temperature produced with a freezing mixture of solid carbon dioxide and acetone (below -80° C.) a brittle solid, apparently non-crystalline, is formed. This product is substantially insoluble in such solvents as ether, benzene, and petroleum ether. It is, however, completely soluble in alcohol and acetone.

The products of this example are entirely soluble in cyanide plating baths up to about three 70 grams per liter. One characteristic of both the final product and the reduced, unseparated reaction mixture is that when used in cyanide-cadmium plating baths they exhibit the property of causing a bright deposit of cadmium. This 75

characteristic serves admirably for the identification of these novel products.

The amaldacets of this example are not chemical compounds, but are mixtures as is evidenced by the fact that portions of the cyanide reaction products are water-soluble and that smaller portions of the products are chloroform-soluble. When used as an addition agent in electroplating cadmium, the water-soluble portion of the cyanide reaction products exhibits the property of promoting the formation of a bright finish on recessed parts of an article. The water insoluble portion seems to exercise its major influence on the brightness of the less recessed parts of the article. The chloroform-soluble fraction is very active as an addition agent, but when used alone it is not satisfactory as it causes streaks and stains on the plated article.

The temperature of the reaction is relatively important as the yield of the product and its activity as an addition agent seem to be greatly influenced thereby. The activity and, of course, the yield of the hydrogenation products of this invention are similarly influenced. The best results seem to be obtained with temperatures between about 45 and 50° C. as used in this example. If lower temperatures are used, there is a decrease in the activity of the product as an addition agent. Below about 30° C. the product rapidly becomes less active with decreases in temperature. If temperatures substantially above 50° are used, the yield of active material is smaller. At about 75° C., for instance, about one-half of the product is an insoluble resin without much value as an addition agent. Generally, I may use temperatures from about 30° C. to about 75° C., though more specifically I prefer to keep the reaction temperature between about 45° and 50° C. so that hydrogenation products of optimum characteristics may be produced from these materials.

The separation by neutralization with acid was accomplished at 50° C., but rigid temperature control is not necessary. Apparently, as soon as the reaction is complete, the reaction product may be heated to rather high temperatures without substantial damage resulting.

In the examples, sulfuric acid is employed for removing excess sodium cyanide by converting it to sodium sulfate which then acts to salt out the addition agent. Obviously other acids can be used which lead to a similar result, and moreover, still other means for removing the excess sodium cyanide will readily occur to those working in the art.

While I may use any of the aldacet as a starting material, I prefer to use aldol because it is readily obtainable commercially at the present time and because it leads to somewhat higher yields than do some of the other aldacet, crotonaldehyde and paraldehyde for instance. Aldol is also advantageously employed by reason of its being less volatile than acetaldehyde and more easily handled than paraldol which is a solid.

As an example of the preparation of an amaldacet from another aldacet, I give the following:

#### Example XI

Eighty parts by weight of acetaldehyde was added slowly to 100 parts by weight of water containing 20 parts by weight of sodium cyanide. The temperature was held between 40° and 50° C. for about one-half hour, at the end of which time the product was allowed to cool.

The resulting amaldacet solution may be hy-

drogenated to produce one product of my invention.

The reaction mixture is preferably concentrated by treatment with dilute sulfuric acid, as described in Example X. The product is substantially identical with the concentrated product of Example X described in detail above.

It is noted that in Example XI a smaller ratio of cyanide to aldehyde was used than in Example X. This seems to lower the yield of active material somewhat. Generally, the best results are obtained when the aldehyde and cyanide are used in substantially molecular proportions, but a latitude is permissible.

If less of the alkali metal cyanide be used, the product will be less active, while if an excess of alkali metal cyanide be used, no particular damage results. When the product is concentrated by neutralizing with dilute sulfuric acid, the excess of cyanide, over that required to form the reaction product, is converted to alkali sulfate and hydrogen cyanide gas, both of which are separated from the product.

The period of time during which the reaction temperature is maintained may be widely varied. If the time be too short, the reaction will not be complete and the product will be of low activity when used as an addition agent for cadmium plating, and its hydrogenation product, similarly, will be of low activity. If the time be too long, a product of excellent activity is obtained, but the yield is low. The time of Example XI represents a practical minimum, and I usually prefer to employ a longer period. In general, the reaction temperature should be maintained for not less than about one-half hour, and I prefer to maintain it for not less than about four hours to obtain a product which, when reduced, yields an addition agent of the highest activity.

The following examples illustrate the preparation of products which have a higher ratio of hydrogen to oxygen than have the amketaldoresins, which reduced products constitute addition agents of my invention:

#### Example XII

To the cyanide reaction product of Example X was added ten grams per liter of zinc dust. The zinc dust in the alkaline solution served, of course, as a reducing agent. After the reaction was complete, the solution was treated with sulfuric acid as in the said Example X to concentrate the resin. Both the reduced cyanide solution and the concentrated product constitute addition agents for cyanide-cadmium plating.

Employing the concentrated product as an addition agent, cyanide-cadmium plating baths were made up as follows:

|                                                       | (1) | Grams per liter |
|-------------------------------------------------------|-----|-----------------|
| Sodium cyanide (NaCN)                                 | 130 |                 |
| Cadmium oxide (CdO)                                   | 43  |                 |
| Sodium sulfate (Na <sub>2</sub> SO <sub>4</sub> )     | 50  |                 |
| Cobalt sulfate (CoSO <sub>4</sub> ·7H <sub>2</sub> O) | 10  | 65              |
| Addition agent                                        | 1.2 |                 |

A plating solution was made up and used in the customary way to plate a number of articles with a cadmium deposit about five-thousandths of an inch thick. After washing with water, the articles were examined and found to have a perfectly smooth, mirror-like finish. It is, of course, very difficult with prior art processes to obtain even a fairly smooth finish when so thick a deposit of cadmium is plated.

This bath displayed good throwing power and a wide bright current density range.

The concentrated product of this example may satisfactorily be employed in widely varying amounts, but I usually prefer to use between about eight-tenths and two grams per liter. The proportion of the amaldacet used above, one and two-tenths grams per liter, is about an optimum under the conditions of this example.

| 10 | (2)                   | Grams per liter |
|----|-----------------------|-----------------|
|    | Cadmium oxide (CdO)   | 25              |
|    | Sodium cyanide (NaCN) | 120             |
| 15 | Addition agent        | 0.6             |

This bath was used for plating several objects at a current density of twenty amperes per square foot. The deposit was extremely bright and smooth. The number of grams of cadmium oxide in the above bath may be varied between fifteen and forty and good results will be obtained. If the bath be too concentrated the deposit will not be entirely satisfactory.

The reduced, dilute solution was used in a similar manner with similar results. About five grams per liter were used with bath (1) and about three grams per liter were used with bath (2).

It is noted that less of the concentrated product was used than of the reaction mixture. The amounts used in each instance, however, represent the amount of product produced from substantially the same amounts of aldol.

The reduced amaldacets are slightly more soluble than the untreated amaldacets, and are more active as addition agents in cyanide-cadmium plating.

#### Example XIII

Following the procedure of the above Example XII, the reaction product of Example XI was hydrogenated. The resulting product and a concentrated product were somewhat more soluble in cyanide-cadmium baths and were effective as addition agents in somewhat smaller concentrations than the corresponding products of Example XI. The addition agents of this example produced results comparable to those of Example XII when used in similar baths at similar concentrations.

#### Example XIV

The crotonaldehyde-monoethanolamine reaction product of Example I was dissolved in an alkali metal cyanide solution, and zinc dust was added to reduce the product. The product gave results comparable with those obtained in Example XII when employed in similar cyanide-cadmium baths.

The other amaldacets shown above in Examples II, III, IV, V, VI, VII, VIII, and IX may similarly be reduced to produce improved addition agents of my invention.

In the foregoing examples, zinc dust was employed as a reducing agent largely because of its convenience, but as will be evident, other reducing agents may satisfactorily be employed. I may, for instance, use a reducing agent such as sodium sulfite. It will be understood that the extent of reduction of the amketaldoresins may be widely varied, the hydrogen presumably saturating some or all of the double bonds.

Some of the reduction products of the heretofore mentioned amaldacets, such as a reduction product of the amaldacet of Example VI, are not

readily soluble in cyanide-cadmium plating baths, and it is desirable that they be dispersed in the baths. With the reduction products of the amketaldoresins generally, likewise, it is expedient to disperse the addition agent if difficulty is encountered in dissolving an optimum quantity. The addition agents may be dispersed and their dissolution aided by adding them to a cyanide-cadmium bath in a suitable solvent, such as alcohol or acetone. It may sometimes be found desirable to reduce the addition agents to a finely divided state, or to use them in conjunction with such dispersing agents as saponin, gum arabic, and sulfite cellulose waste.

While my addition agents are effective in any customary cyanide bath, I prefer to use baths of the kind set forth in U. S. Patent 1,681,509 to Mr. Leon R. Westbrook and as shown in Example XII, bath (1). These baths are of the cyanide type, and contain a small amount of a compound of a metal of the iron group having an atomic weight greater than fifty-eight. The details as to the formulation and use of these baths may be found in the said Patent 1,681,509 and need not be duplicated here.

The plating baths of the said Patent 1,681,509 are modified, as shown above, only by employing my novel addition agents in lieu of the addition agents, goulac, dextrin, starch, etc., mentioned therein. While the plating processes described in the said Patent 1,681,509 lead to a bright, hard, dense, and smooth deposit of cadmium, and while the invention therein described and claimed has been widely accepted by the art because of its merit, the substitution of my addition agents for those in the patent results in a cadmium deposit of even greater smoothness, uniformity, and brightness.

Of course, I may use other compounds of metals of the iron group having an atomic weight greater than fifty-eight, such as nickel, copper, etc., as disclosed in the heretofore mentioned Patent 1,681,509, but the use of cobalt compounds, as in Example XII, bath (1), has led to the best results.

I desire that it be clearly understood that the whole disclosure of the heretofore mentioned Patent 1,681,509, as well as that of U. S. Patent 1,564,413 to Clayton M. Hoff, cited therein, is to be considered, in its entirety, as an integral part of my disclosure, as my novel addition agents co-act with the cyanide-metal compound baths therein to produce a result unexpected from an examination of the attributes of either of my addition agents or the baths of the said patent, for baths of such high concentration cannot be used to advantage without the metal compounds added by Westbrook.

While I have discussed above the use of baths of the Westbrook type, I do not wish to be limited thereto. I prefer to use them because of certain commercial considerations, and because they may be more concentrated, but excellent results are obtainable with other types of baths such as the one shown, for instance, in Example XII, bath (2).

In the foregoing, the amketaldoresins derived by reacting an aldacet with ammonia, an amine, or cyanide have been discussed in some detail with reference to their preparation, their properties, and the application of their reduction products as addition agents in cyanide-cadmium plating. The products thus considered above are, in many respects, typical of those obtainable by the reduction of amketaldoresins.

The amaldacets are, of course, derived from certain aliphatic ketaldones: the aldecets. Below are discussed typical amketaldoresins derived from other aliphatic ketaldones and from 5 carbocyclic ketaldones.

The following typical aliphatic ketaldones were tried as starting materials for the production of amketaldo-resins which could be hydrogenated according to my invention. The aldecets are included for purposes of comparison. The compounds in the respective lists are given in about 10 the order of their desirability as starting materials.

#### Aldehydes

- 15 1. Aldol
- 2. Acetaldehyde
- 3. Crotonaldehyde
- 4. Paradol
- 5. Propionaldehyde
- 6.  $\alpha$ -ethyl  $\beta$ -propyl acrolein
- 7. Butyraldehyde
- 8. Acrolein
- 9. Citral
- 25 10. Citronellal
- 11. Hexadecocic aldehyde
- 12. Isobutylaldehyde

#### Ketones

- 30 1. Diethyl ketone
- 2. Methyl n-propyl ketone
- 3. Methyl ethyl ketone
- 4. Diacetyl
- 5. Light acetone oil
- 6. Heavy acetone oil
- 35 7. Isobutyl ketone
- 8. Acetone
- 9. Iso amyl ketone

Considering more specifically the preparation 40 of amketaldoresins from the above aliphatic ketaldones, the following specific examples are given:

#### Example XV

45 Equimolecular proportions of monoethanolamine and propionaldehyde were reacted at room temperature. A soluble resin was obtained which, when reduced and employed in baths such as those of Example XII, displayed activity as an addition agent but was none too satisfactory.

#### Example XVI

50 Methyl ethyl ketone was treated at room temperature with gaseous ammonia. The resulting reaction product, when hydrogenated, displayed 55 activity as an addition agent in cyanide-cadmium plating baths.

#### Example XVII

60 Five parts by weight of propionaldehyde were mixed with three parts by weight of sodium cyanide and ten parts by weight of water. The mixture was maintained at a temperature of about 50° C. for two hours and then allowed to cool. 65 There was a change in the appearance of the mixture during the reaction period. The reaction product was a homogeneous, mobile liquid, light yellow in color.

70 The addition agent of this example was reduced and used in a cyanide-cadmium bath such as that of Example XII, bath (1), the addition agent of this example being used at a concentration of about 1.4 cc. per liter in lieu of the concentrated addition agent of Example XII. A 75 bright, lustrous cadmium deposit was obtained,

and the bath was characterized by good throwing power and a relatively wide bright current density range.

#### Example XVIII

5

Diethyl ketone was treated with sodium cyanide according to the procedure of Example XVII, and the reaction product permitted to stand a few days. The reaction mixture separated into two layers: a colorless lower layer, 10 which is probably sodium cyanide solution, and an upper layer light yellow in color. While I may use both layers mixed together, I prefer to separate, and use, the upper layer.

The yellow upper layer was reduced with zinc 15 dust and used in cyanide-cadmium baths of the type shown in Example XII, bath (1), at an optimum concentration of 5 cc. per liter. Excellent results were obtained. The colorless lower layer, when reduced, displayed no appreciable activity as an addition agent. 20

#### Example XIX

25

Methyl ethyl ketone was treated with sodium cyanide according to the procedure of Example XVII and then allowed to stand a few days. The reaction mixture separated into a lower, light yellow layer, and a small upper layer, dark red in color. Again I may use the mixture, 30 but I prefer to use the upper layer.

The upper, dark red layer was reduced with zinc dust and used at a concentration of 6 cc. per liter in a cyanide-cadmium bath of the type shown in Example XII, bath (1), with fair results. The lower, light yellow layer, when reduced, 35 was not substantially effective as an addition agent in cyanide-cadmium plating.

#### Example XX

40

Diacetyl was treated with sodium cyanide according to the procedure of Example XVII, and a homogeneous liquid was obtained.

The diacetyl-cyanide reaction product was reduced and then employed at a concentration of 2 cc. per liter in a bath of the type shown in Example XII, bath (1), with good results. 45

#### Example XXI

50

Methyl n-propyl ketone was treated with sodium cyanide according to the procedure of Example XIX. A colorless upper layer and a colorless lower layer were obtained. Again I may use the reaction mixture, but I prefer to use the upper layer.

The upper layer was reduced, and was found to be a good addition agent when employed at a concentration of 6 cc. per liter in a cyanide-cadmium bath of the type shown in Example XII, bath (1). The lower layer, when reduced, 60 showed no substantial effect as an addition agent in cyanide-cadmium baths. 55

#### Example XXII

65

Acetone was treated with sodium cyanide according to the procedure of Example XIX. After standing three weeks, a light red lower layer and a dark red upper layer formed. I may use the mixture, but I prefer to hydrogenate the upper layer separately.

The light red lower layer, after reduction, was somewhat effective as an addition agent in a cyanide-cadmium bath of the type shown in Example XII, bath (1). When reduced and used 75 as an addition agent in a bath of the same type, 75

the dark red upper layer was found quite satisfactory at a concentration of 18 cc. per liter.

*Example XXIII*

5 Butyraldehyde was treated with sodium cyanide according to the procedure of Example XIX. The two layers which formed may both be reduced to produce addition agents, and I may use either or the mixture.

10 The lower layer, after reduction, gave good results as an addition agent at a concentration of 15 cc. per liter in a cyanide-cadmium bath of the type shown in Example XII, bath (1). The upper layer, after reduction, produced even better results at a concentration of only 5 cc. 15 per liter in a cyanide-cadmium bath of the same type.

*Example XXIV*

20 Hexadecoic aldehyde was treated with sodium cyanide according to the procedure of Example XVII, the mixture of aldehyde and cyanide being maintained at about 50° C. for four hours. The reaction mixture was allowed to stand overnight and was found to have separated with a top 25 layer of nearly black cyanide reaction product. It is noted that the original aldehyde was light yellow in color.

30 The lower layer, even when reduced, had no appreciable effect as an addition agent in a cyanide-cadmium bath of the type shown in Example XII, bath (1). The upper layer, after reduction, was rather difficultly soluble, but at its optimum concentration of 5 cc. per liter, it 35 served as an addition agent in a cyanide-cadmium bath of the same type. The agent produced from the top layer being poorly soluble, it should be dispersed in the bath after the manner hereinbefore suggested.

40 When aliphatic ketaldones are used as starting materials, a ketaldone should be selected which contains at least two carbon atoms. Formaldehyde, with but one carbon atom, stands in a unique position with respect to aldehydes 45 generally. Its dissimilarity to the other aldehydes is, of course, generally recognized.

Two hundred cubic centimeters of a forty per cent solution of formaldehyde was slowly added to a solution of sixty grams of sodium cyanide 50 in eighty cubic centimeters of water. The temperature rose rapidly, and the reaction vessel was cooled to maintain a temperature of about 45° to 50° C. After about two-thirds of the formaldehyde was added, the addition of the remaining one-third produced no appreciable effect. After about ten minutes, however, the reaction mixture became hot and it was necessary 55 to cool it. After the reaction was complete, a dark colored product was obtained. This product was tried as an addition agent, using from one to ten grams per liter, in a bath of the type shown in Example XII, bath (1), and it was found that the product had only a slight effect on the character of cadmium deposit. No substantial improvement resulted from reduction 60 of the agent.

In view of the difference between formaldehyde and other aldehydes, one would expect 65 formaldehyde to behave differently as a starting material for the production of addition agents. As addition agents prepared from formaldehyde are of a different order of effectiveness and are of a different character from the agents prepared from other aldehydes, I prefer to employ ketaldones which have more than one carbon atom.

As the aliphatic ketaldones contain more and more carbon atoms, they appear to become less desirable as starting materials for the production of amketaldoresins. Citral and citronella, for example, with nine carbon atoms are quite satisfactory as starting materials for the production of addition agents, but the agents tend to be somewhat insoluble. They may, of course, be dispersed in the bath, but it is ordinarily preferable that the agents be readily soluble in the 10 amounts required.

Above about nine carbon atoms the aliphatic ketaldones become somewhat less desirable as starting materials. Hexadecoic aldehyde, for instance, with sixteen carbon atoms led to the 15 production of a relatively insoluble, though operative, amketaldoresin. I prefer, accordingly, to employ aliphatic ketaldones containing between two and nine carbon atoms. This terminology includes acetaldehyde, for example, as a 20 two carbon atom compound and citral as a nine carbon atom compound. I especially prefer to employ those aliphatic ketaldones of two to nine carbon atoms which contain no more than two hydroxyl groups.

I have found that it is not desirable that the aliphatic ketaldones contain carboxyl groups. Moreover, the elements sulfur and nitrogen are 30 preferably absent from the aliphatic ketaldones which I employ as starting materials for the production of amketaldoresins. I especially prefer to use aliphatic ketaldones which contain only carbon, hydrogen, and oxygen, and in which the hydrogen-oxygen ratio is higher than that of water.

While, as is noted above, I prefer that the aliphatic ketaldones which I employ as starting materials contain no more than two hydroxyl groups, and, more specifically, that they have a higher ratio of hydrogen to oxygen than that of water, it is, nevertheless, within the scope of my present invention to use such ketaldones as ketoses and aldoses.

When carbohydrates which contain an aldehyde or ketone group are treated with an amo 45 or with an alkali metal cyanide and then reduced, products similar to those above may, with some difficulty, be prepared. The reduced amketaldoresins thus produced, however, are of a different order of effectiveness than the preferred reduced 50 amketaldoresins.

The following example illustrates the production of a reduced amketaldoresin from a carbohydrate which contains a ketaldonyl group.

*Example XXV*

Glucose was treated with an alkali metal cyanide by adding 12.3 grams of glucose to a cyanide solution made by adding 3.3 grams of sodium cyanide to 10 cubic centimeters of water. The 60 mixture was maintained at about 45° to 50° C. for eighteen hours and was agitated intermittently. During the period of treatment, a faint odor of ammonia was observed.

At the end of the eighteen hours, the product was a dark red-brown, viscous liquid. This product was allowed to stand for about five hours, and then four and one-half cubic centimeters of dilute sulfuric acid was added thereto. This quantity 70 of sulfuric acid was an excess over the amount required to react with the unreacted sodium cyanide.

When the acid was added, some heat was evolved, and there was foaming of the product.

After the foam subsided, the product was a clear, red-brown, homogeneous liquid.

The product produced was reduced with zinc dust and employed as an addition agent in cyanide-cadmium baths of the type shown in Example XII in various concentrations up to ten grams per liter. The addition agent effected a considerable change in the character of the cadmium deposits, but was none too satisfactory. It is noted that the baths containing the addition agent were reddish-yellow in color.

For purposes of direct comparison, glucose was employed as an addition agent for cyanide-cadmium baths of the same type and in the same concentrations as were the products of this example. Glucose itself was much less effective than its reduced cyanide-reaction product. It is noted that the baths containing glucose were light-yellow in color.

20 The reduced amketaldoresins prepared from the aliphatic ketaldones have been discussed above in some detail, and it is now proposed to discuss briefly the preparation of reduced amketaldoresins from carbocyclic ketaldones.

25 The reduced amketaldoresins may be prepared by the treatment of carbocyclic ketaldones with an amo or cyanide according to procedures similar to those above discussed.

30 The following carbocyclic ketaldones, tried as starting materials for the production of amketaldoresins, are listed in the approximate order of their desirability.

1. Cyclohexanone
2. Methyl cyclohexanone
3. Benzoin
4. Benzaldehyde
5. Anisic aldehyde
6. Cinnamic aldehyde
7. Quinone
8. Vanillin
9. Ortho-ortho dicarboxy benzoin

In order more fully to describe the production of the reduced amketaldoresins from the carbocyclic ketaldones, the following illustrative examples are given:

#### Example XXVI

50 Equimolecular proportions of monoethanolamine and benzaldehyde were reacted to room temperature, and the reaction mixture reduced. The product displayed activity as an addition agent in a cyanide-cadmium plating bath of the type shown in Example XII, bath (1).

#### Example XXVII

Gaseous ammonia was passed into benzaldehyde until the reaction was complete. The amketaldoresin produced, after reduction, was found 60 to have activity as an addition agent in a cyanide-cadmium bath of the type shown in Example XII, bath (1).

#### Example XXVIII

65 Benzaldehyde was treated at 50° C. for several hours with an excess of sodium cyanide solution. The cyanide solution contained three parts by weight of sodium cyanide to ten parts by weight of water. As the benzaldehyde was added to the 70 cyanide solution a precipitate of some relatively insoluble material formed. After a few hours most of this precipitate had dissolved. The reaction mixture, after reduction, was employed quite successfully with a cyanide-cadmium bath of the 75 type shown in Example XII, bath (1).

Benzaldehyde is known to form benzoin in alkaline solution according to the following:



Accordingly, I believe that the precipitate noted above was benzoin, and that on further treatment at 50° C. some further change took place 10 which resulted in the formation of a more soluble compound. The benzoin may have reacted with ammonia, or cyanide, condensed further, or perhaps all.

#### Example XXIX

Benzoin was treated as in Example XXVIII, and, after some time, the product was reduced and a satisfactory addition agent was obtained. By dissolving the benzoin in alcohol and then treating the alcohol solution with cyanide, the final product was made more quickly. In the latter procedure the alcohol was removed from the reaction product by distillation. The products obtained by treating the benzoin with cyanide, and reducing, were quite satisfactory addition agents in cyanide-cadmium baths of the type shown in Example XII, bath (1).

#### Example XXX

30 As the starting materials, benzaldehyde and benzoin, are difficultly soluble, I added two carboxyl groups to benzoin thus:



40 This ortho-ortho dicarboxy benzoin was much more soluble than benzoin, but it was none too satisfactory as a starting material for the production of addition agents. Ortho-ortho dicarboxy benzoin was treated with cyanide, as in the above examples, and, after reduction, the product was found to possess some activity as an addition agent in cyanide-cadmium baths.

45 The other carbocyclic compounds above listed may similarly be treated with an amo or cyanide according to the above procedures with good results. It is noted that instead of using methyl cyclohexanone, I may use other alkyl substituted cyclohexanones. I may, of course, use more than one alkyl substituent.

55 While generally I may advantageously employ any carbocyclic ketaldone, I prefer to use as starting materials ketaldones which do not contain a carboxyl group and which do not contain sulfur. Moreover, carbocyclic ketaldones which do not contain nitrogen are ordinarily preferred, because while Michler's ketone, for instance, responds to my broadest definition, it is none too satisfactory a starting material. Specifically, I prefer to employ carbocyclic ketaldones which contain only carbon, hydrogen, and oxygen and in which the hydrogen-oxygen ratio is greater than that of water.

60 The foregoing discussion of the aromatic ketaldones is limited to a preferred group, the carbocyclic ketaldones. It will be understood, however, that my invention in its broad aspects includes the use of cyclic ketaldones generally. I may, for instance, use heterocyclic ketaldones 65 as starting materials for the preparation of addition agents for cyanide-cadmium plating baths.

The following example illustrates the practice of my invention using a heterocyclic ketaldone:

*Example XXXI*

5 Six and one-half grams of freshly distilled furfural was added to a sodium cyanide solution made up of 3.3 grams of sodium cyanide in 10 cubic centimeters of water. Quickly there was produced a red, heterogeneous mixture which was 10 then maintained for six hours at 45° to 50° C. During the reaction period, a faint odor of ammonia was observed. At the end of the six hours, the mixture had reacted to form a black, tarry, lower layer and a brown, supernatant liquid. 15 The black lower layer, after reduction, is effective as an addition agent.

The reaction mixture obtained above, before reduction, was treated with an excess of dilute sulfuric acid over that required to react with 20 excess sodium cyanide, after the procedure of Example X. Upon the addition of acid, a violent reaction took place, and a small amount of a black, liquid tar separated from the upper layer and joined the tar already at the bottom of the 25 reaction receptacle.

The mixture of tars was employed, after reduction, as an addition agent in cyanide-cadmium baths of the type above shown in Example XII. The baths were of a reddish color. Excellent 30 results were obtained, but the agent of this example did not cause the baths to display as extended a bright current density range as did the agents of Example X.

The agents of this example are rather difficultly soluble, and it is preferred to add them to 35 cyanide-cadmium baths in a suitable solvent such as alcohol. An optimum effect appears to be obtained when from about one-half to two grams per liter of the agents are used.

40 It will be understood that the conditions for the preparation of the furfural-cyanide products of this example may be widely varied. It is preferable that about an equivalent amount, or a slight excess of sodium cyanide be used. It should 45 be noted in this connection that a great excess of cyanide is not satisfactory as, in effect, the furfural would be present in too small a concentration for the proper reactions to take place.

Furfural was employed as an addition agent for 50 cyanide-cadmium baths, of the type used in Example XII, in various amounts up to about ten grams per liter. After standing for several hours, the baths became very dark in color, and appeared black. By strong transmitted light, a 55 small sample of one such bath appeared to have a dark, wine color. While furfural, in relatively large amounts, displayed some activity as an addition agent, it was very much less effective than the reduced furfural-cyanide products of this example.

60 It will be understood therefore that in the production of amketaldoresins no such great departure from equimolecular proportions should be made. It will also be evident that the reacting materials should not be too dilute.

In order conveniently to merchandise my novel 65 addition agents, I may incorporate them with the dry ingredients employed to make up a plating bath. The resulting dry mixture can then 70 be packaged and sold to the consumer who needs only to dissolve the mixture in water for use. Again, I may find it desirable to incorporate the addition agent with only one or a few of the ingredients and let the consumer add the other 75 ingredients. Frequently, of course, it will be de-

sirable to merchandise the novel addition agents as such.

While I have disclosed a number of specific cyanide-cadmium baths heretofore, it will be understood that I do not intend to be limited thereby and that the teachings of my invention may be applied to cyanide-cadmium baths generally. 5

It will also be understood that I do not intend to be limited to the specific reduced amketaldoresins above disclosed, as numerous other such compositions can readily be prepared by those skilled in the art according to the principles of my invention. 10

I claim:

1. A cyanide-cadmium plating composition containing a hydrogenated amketaldoresin, the extent of hydrogenation being of the magnitude of the hydrogenation obtainable by the addition of zinc dust to the amketaldoresin in alkaline 20 solution, an amketaldoresin being, as herein set forth, a pre-reacted compound prepared by reacting a ketaldone with an amo in alkaline solution. 20

2. A cyanide-cadmium plating composition containing a hydrogenated amketaldoresin derived from a carbocyclic ketaldone, the extent of hydrogenation being of the magnitude of the hydrogenation obtainable by the addition of zinc dust to the amketaldoresin in alkaline solution, an amketaldoresin being, as herein set forth, a 30 pre-reacted compound prepared by reacting a ketaldone with an amo in alkaline solution. 25

3. A cyanide-cadmium plating composition containing a hydrogenated amketaldoresin derived from an aliphatic ketaldone, the extent of hydrogenation being of the magnitude of the hydrogenation obtainable by the addition of zinc dust to the amketaldoresin in alkaline solution, an amketaldoresin being, as herein set forth, a 35 pre-reacted compound prepared by reacting a ketaldone with an amo in alkaline solution. 40

4. A cyanide-cadmium plating composition containing a hydrogenated amketaldoresin derived from an aliphatic ketaldone which contains only carbon, hydrogen, and oxygen, which 45 has no less than two and no more than nine carbon atoms, and in which the ratio of hydrogen to oxygen is greater than that of water, the extent of hydrogenation being of the magnitude of the hydrogenation obtainable by the addition of zinc dust to the amketaldoresin in alkaline solution, an amketaldoresin being, as herein set forth, a 50 pre-reacted compound prepared by reacting a ketaldone with an amo in alkaline solution.

5. A cyanide-cadmium plating composition 55 containing a hydrogenated reaction product of an amo with an aliphatic aldehyde selected from the group consisting of aldol, acetaldehyde, croto-aldehyde, and paraldol, the extent of hydrogenation being of the magnitude of the hydrogenation obtainable by the addition of zinc dust to the reaction product in alkaline solution.

6. A cyanide-cadmium plating composition containing a hydrogenated reaction product of an amo with aldol, the extent of hydrogenation 65 being of the magnitude of the hydrogenation obtainable by the addition of zinc dust to the reaction product in alkaline solution.

7. A cyanide-cadmium plating composition containing a hydrogenated reaction product of 70 an alkali metal cyanide with a ketaldone, the extent of hydrogenation being of the magnitude of the hydrogenation obtainable by the addition of zinc dust to the reaction product in alkaline solution. 75

8. A cyanide-cadmium plating composition containing a hydrogenated reaction product of an alkali metal cyanide with a carbocyclic ketaldone, the extent of hydrogenation being of the magnitude of the hydrogenation obtainable by the addition of zinc dust to the reaction product in alkaline solution.

9. A cyanide-cadmium plating composition containing a hydrogenated reaction product of an alkali metal cyanide with an aliphatic ketaldone, the extent of hydrogenation being of the magnitude of the hydrogenation obtainable by the addition of zinc dust to the reaction product in alkaline solution.

10. A cyanide-cadmium plating composition containing a hydrogenated reaction product of an alkali metal cyanide with an aliphatic ketaldone which contains only carbon, hydrogen, and oxygen, which has no less than two and no more than nine carbon atoms, and in which the ratio of hydrogen to oxygen is greater than that of water, the extent of hydrogenation being of the magnitude of the hydrogenation obtainable by the addition of zinc dust to the reaction product in alkaline solution.

11. A cyanide-cadmium plating composition containing a hydrogenated reaction product of an alkali metal cyanide with an aldacet, the extent of hydrogenation being of the magnitude of the hydrogenation obtainable by the addition of zinc dust to the reaction product, an aldacet being, as herein set forth, one of the aldehyde equilibrium products which result when acetaldehyde is put in alkali metal cyanide solution.

12. A cyanide-cadmium plating composition containing a hydrogenated reaction product of an alkali metal cyanide with an aliphatic aldehyde selected from the group consisting of aldol, acet-aldehyde, crotonaldehyde, and paraldol, the extent of hydrogenation being of the magnitude of the hydrogenation obtainable by the addition of zinc dust to the reaction product in alkaline solution.

13. A cyanide-cadmium plating composition containing a hydrogenated reaction product of an alkali metal cyanide with aldol, the extent of

hydrogenation being of the magnitude of the hydrogenation obtainable by the addition of zinc dust to the reaction product in alkaline solution.

14. A cyanide-cadmium plating composition containing a hydrogenated amketaldoresin and a small amount of a metal of the iron group having an atomic weight greater than fifty-eight, the extent of hydrogenation being of the magnitude of the hydrogenation obtainable by the addition of zinc dust to the amketaldoresin in alkaline solution, an amketaldoresin being, as herein set forth, a pre-reacted compound prepared by reacting a ketaldone with an amo in alkaline solution.

15. In a process for the electrodeposition of cadmium, the step comprising depositing cadmium from a cyanide-cadmium bath in the presence of an addition agent comprising a hydrogenated amketaldoresin, the extent of hydrogenation being of the magnitude of the hydrogenation obtainable by the addition of zinc dust to the amketaldoresin in alkaline solution, an amketaldoresin being, as herein set forth, a pre-reacted compound prepared by reacting a ketaldone with an amo in alkaline solution.

16. In a process for the electrodeposition of cadmium, the step comprising depositing cadmium from a cyanide-cadmium bath in the presence of an addition agent comprising a hydrogenated reaction product of an alkali metal cyanide with a ketaldone, the extent of hydrogenation being of the magnitude of the hydrogenation obtainable by the addition of zinc dust to the reaction product in alkaline solution.

17. In a process for the electrodeposition of cadmium, the step comprising depositing cadmium from a cyanide-cadmium bath in the presence of an addition agent comprising a hydrogenated reaction product of an alkali metal cyanide of an aliphatic aldehyde selected from the group consisting of aldol, acetaldehyde, crotonaldehyde, and paraldol, the extent of hydrogenation being of the magnitude of the hydrogenation obtainable by the addition of zinc dust to the reaction product in alkaline solution.

GEORGE LUTZ.